

Dec. 2, 1930.

C. W. MAYER ET AL

1,783,442

RECORDING PAPER

Filed Feb. 4, 1928



INVENTORS  
Charles W. Mayer  
BY Thureott W. Siller  
Cyrnston & Griffith  
their ATTORNEYS

## UNITED STATES PATENT OFFICE

CHARLES W. MAYER AND EVERETT F. SILLER, OF ROCHESTER, NEW YORK

## RECORDING PAPER

Application filed February 4, 1928. Serial No. 251,998.

This invention relates to recording paper. It has for an object the preparation of a new and improved type of such paper.

More particularly the invention relates to 5 that form of recording paper, for example, known as non-carbon paper which is adapted to form in itself a permanent record of impressions thereon, and which in this case consists of a paper base or stock preferably colored, which is coated with a waxy compound 10 transparent when liquid but translucent and preferably white when crystallized.

Further objects comprise the treatment of 15 the surface so as to reduce susceptibility to abrasion under friction without affecting the sensitivity of the paper for recording purposes and to remove tackiness or stickiness.

To these and other ends the invention resides in certain improvements and combinations of parts, all as will be hereinafter more fully described, the novel features being pointed out in the claims at the end of the specification.

## In the drawings:

25 Fig. 1 is a perspective view of a sample of the finished paper with a portion of the coating lifted to show the base, and

Fig. 2 is a section through the sample of the finished paper.

30 The recording or non-carbon paper forming the subject matter of this invention consists, as above indicated, of a paper base, preferably covered, and covered by a compound transparent while liquid, but translucent and preferably white when crystallized.

35 Characters may be recorded on the paper by primary or secondary impression or by heat, that is by mechanically displacing or compacting the coating as by a stylus or by im- 40 pact of a typewriter key, or by rendering the coating locally transparent, for instance, by the use of localized heat. This allows the paper base to appear through the coating, the exposed portions of the base forming the de- 45 sired characters.

One combination which has been successfully used by applicants is that of a dark colored paper base with a coating thereon, formed of a mixture of a fatty acid and 50 water-insoluble soaps, with a small amount

of clay, and a suitable amount of volatile solvent, such as alcohol, gasoline, or carbon tetrachloride.

A specific example of such a compound is given in the following formula:

16 lbs. stearic acid, 1 lb. aluminum palmitate, 3 lbs. aluminum oleate,  $\frac{1}{2}$  lb. clay, sufficient alcohol to give the desired consistency.

It will be understood that the proportions of the above formula may be varied considerably to secure the desired characteristics of the finished product. For example, the aluminum oleate largely controls the sensitivity of the emulsion, and may be varied from one-half pound to five pounds to secure 60 parts of varying sensitivity for different uses.

The stearic acid is the base of this formula and is largely instrumental in securing the crystallized condition which makes the coating translucent. However, if used alone the 70 stearic acid forms large coarse crystals and the aluminum palmitate is added to secure a finer crystallization and also to raise the viscosity of the melted compound. The clay is simply a filler and may be used in various 75 amounts or eliminated altogether if desired. The volatile solvent is used as a means of controlling crystallization, and to reduce the mixture to a consistency that can be handled readily on any coating machine.

The use of variations of the above formula and the substitution of materials of equivalent properties are contemplated and intended to be covered by the claims appended hereto.

85 The paper coated with the coating material may be used on recording instruments etc. but at this stage it is easily abraded by friction and is difficult to handle in quantity because of its sticky surface. In order to obviate this difficulty, applicants conceived the idea of coating the sensitized surface with an inert unctuous powder such as talc, and have found that this procedure entirely overcomes this difficulty, and moreover increases the 90 whiteness of the film and affords general protection against atmospheric conditions.

95 After this finishing operation, the surface is entirely free from tackiness, and the resistance to abrasion under friction in han- 100

dling has been found to be very greatly increased without affecting the sensitivity of the paper for recording purposes.

5 To recapitulate, applicants' paper is provided with a translucent crystallized compound having a protected surface. The application of the coating and of the powder may be done on any suitable coating and dusting machines.

10 Since the embodiment of the invention herein disclosed may be variously modified, and since other embodiments thereof might be made without departing from the essence of the invention, this disclosure is to be taken 15 as illustrative only and not as limiting the scope of the invention as pointed out in the claims appended hereto.

We claim as our invention:

20 1. A recording paper consisting of a deeply colored stock, covered with a waxy crystallized coating of contrasting color and an outer layer of inert powder.

25 2. A recording paper consisting of a dark paper base, covered with a compound comprising a crystallized mixture of a fatty acid and water-insoluble soaps, with a small amount of inert loading material, and coated with a thin layer of unctuous powder.

30 3. A recording paper consisting of a dark paper base, covered with a compound comprising a mixture of the following ingredients in approximately the following proportions: stearic acid 16 lb., aluminum palmitate 1 lb., aluminum oleate  $\frac{1}{2}$  to 5 lb.

35 4. A recording paper consisting of a dark paper base, covered with a compound comprising a mixture of the following ingredients in approximately the following proportions: stearic acid 16 lb., aluminum palmitate 1 lb., aluminum oleate  $\frac{1}{2}$  to 5 lb., clay  $\frac{1}{2}$  lb. and coated with an adherent layer of powdered talc or the like.

40 45 5. A recording paper comprising a paper base covered with a waxy crystallized coating of a color contrasting with the color of said base and an outer layer of inert powder.

CHARLES W. MAYER.  
EVERETT F. SILLER.